

**PHOTOGRAPHIC SENSITIZING DYES AND EMULSIONS CONTAINING THEM**

Leslie G. S. Brooker and Donald W. Heseltine, Rochester, N.Y., assignors to Eastman Kodak Company, Rochester, N.Y., a corporation of New Jersey

No Drawing. Application May 21, 1956  
Serial No. 585,946

13 Claims. (Cl. 96—102)

This invention relates to certain cyanine dyes useful in optically sensitizing photographic silver halide emulsions, and to photographic silver halide emulsions sensitized with these cyanine dyes.

The dyes of our invention can advantageously be represented by the following general formula:



wherein R represents an alkyl group, such as methyl, ethyl, n-propyl, n-butyl, carbethoxymethyl, benzyl (phenylmethyl), etc. (e.g., an alkyl group containing from 1 to 4 carbon atoms), n and d each represents a positive integer of from 1 to 2, Q represents the atoms necessary to complete a cyclohexene ring, R<sub>1</sub> represents a cyano group or a carbalkoxyl group, such as carbomethoxyl, carbethoxyl, etc. (e.g., a lower alkoxy carbonyl group), and Z represents the non-metallic atoms necessary to complete a heterocyclic nucleus containing from 5 (n is 1) to 6 (n is 2) atoms in the heterocyclic ring, such as those selected from the group consisting of those of the thiazole series (e.g., thiazole, 4-methylthiazole, 5-methylthiazole, 4-phenylthiazole, 5-phenylthiazole, 4,5-dimethylthiazole, 4,5-diphenylthiazole, 4-(2-thienyl)thiazole, etc.), those of the benzothiazole series (e.g., benzothiazole, 4-methylbenzothiazole, 5-methylbenzothiazole, 6-methylbenzothiazole, 4-phenylbenzothiazole, 5-phenylbenzothiazole, 4-methoxybenzothiazole, 5-methoxybenzothiazole, 6-methoxybenzothiazole, 4-ethoxybenzothiazole, 5-ethoxybenzothiazole, tetrahydrobenzothiazole, 5,6-dimethoxybenzothiazole, 5,6-dioxymethylenebenzothiazole, 5-hydroxybenzothiazole, 6-hydroxybenzothiazole, etc.), those of the naphthothiazole series (e.g., naphtho[2,1]thiazole, naphtho[1,2]thiazole), 5-methoxynaphtho[1,2]thiazole, 5-ethoxynaphtho[1,2]thiazole, 7-methoxynaphtho[2,1]thiazole, 8-methoxynaphtho[2,1]thiazole, etc.), those of the thianaphtho-7',6',4,5-thiazole series (e.g., 4'-methoxythianaphtho-7',6',4,5-thiazole, etc.), those of the oxazole series (e.g., 4-methyloxazole, 5-methyloxazole, 4-phenyloxazole, 4,5-diphenyloxazole, 4-ethyloxazole, 4,5-dimethyloxazole, 5-phenyloxazole, etc.), those of the benzoxazole series (e.g., benzoxazole, 5-phenylbenzoxazole, 5-methylbenzoxazole, 6-methylbenzoxazole, 5,6-dimethylbenzoxazole, 4,6-dimethylbenzoxazole, 5-methoxybenzoxazole, 6-methoxybenzoxazole, 5-ethoxybenzoxazole, 5-hydroxybenzoxazole, 6-hydroxybenzoxazole, etc.), those of the naphthoxazole series (e.g., naphth[2,1]oxazole, naphth[1,2]oxazole, etc.), those of the selenazole series (e.g., 4-methylselenazole, 4-phenylselenazole, etc.), those of the benzoselenazole series (e.g., benzoselenazole, 5-methoxybenzoselenazole, 5-hydroxybenzoselenazole, tetrahydrobenzoselenazole, etc.), those of the naphthoselenazole series (e.g., naphtho[2,1]selenazole, naphtho[1,2]selenazole, etc.), those of the thiazoline series (e.g., thiazoline, 4-methylthiazoline, etc.), those of the 2-quinoline series (e.g., quinoline, 3-methylquinoline, 5-methylquin-

line, 7-methylquinoline, 8-methylquinoline, 6-methoxyquinoline, 6-ethoxyquinoline, 6-hydroxyquinoline, 8-hydroxyquinoline, etc.), those of the 4-quinoline series (e.g., quinoline, 6-methoxyquinoline, 7-methylquinoline, 8-methylquinoline, etc.), those of the 1-isoquinoline series (e.g., isoquinoline, 3,4-dihydroisoquinoline, etc.), those of the 3,3-dialkylindolenine series (e.g., 3,3-dimethylindolenine, 3,3,5-trimethylindolenine, 3,3,7-trimethylindolenine, etc.), those of the 2-pyridine series (e.g., pyridine,

- 5 10 15 20 25 30 35 40 45 50 55 60 65 70
- 3-methylpyridine, 4-methylpyridine, 5-methylpyridine, 6-methylpyridine, 3,4-dimethylpyridine, 3,5-dimethylpyridine, 3,6-dimethylpyridine, 4,5-dimethylpyridine, 4,6-dimethylpyridine, 3-hydroxypyridine, 4-hydroxypyridine, 5-hydroxypyridine, 6-hydroxypyridine, 3-phenylpyridine, 4-phenylpyridine, 6-phenylpyridine, etc.), those of the 4-pyridine series (e.g., 2-methylpyridine, 3-methylpyridine, 2,3-dimethylpyridine, 2,5-dimethylpyridine, 2,6-dimethylpyridine, 2-hydroxypyridine, 3-hydroxypyridine, etc.), those of the benzimidazole series (e.g., benzimidazole, 5-chlorobenzimidazole, 5,6-dichlorobenzimidazole, 1,7-trimethylenebenzimidazole, 5-acetylbenzimidazole, 5-ethylcarbamylbenzimidazole, etc.), those of the pyrrolidine series (e.g., pyrrolidine, etc.), those of the acenaphtho[1,2]thiazole series (e.g., acenaphtho[1,2]thiazole, etc.), etc. When Z represents the non-metallic atoms necessary to complete a pyrrolidine nucleus, R can represent an aryl group, such as phenyl, tolyl, etc. (e.g., a monocyclic aryl group of the benzene series).

Accordingly, it is an object of our invention to provide a new class of optical sensitizing dyes. Another object is to provide photographic silver halide emulsions sensitized with these new dyes. Still another object is to provide methods for making these new dyes. Other objects will become apparent from a consideration of the following description and examples.

The instant invention provides methods for making the dyes represented by Formula I above by condensing a cyclammonium quaternary salt selected from those represented by the following general formula:



wherein R, n and Z each have the values given above, X represents an acid radical, such as chloride, bromide, iodide, thiocyanate, p-toluenesulfonate, benzenesulfonate, ethylsulfate, etc., and R<sub>2</sub> represents an alkylmercapto group (e.g., methylmercapto, ethylmercapto, etc.), and arylmercapto group (e.g., phenylmercapto, tolylmercapto, etc.), or a  $\beta$ -acylanilidovinyl group (e.g.,  $\beta$ -acetanilidovinyl,  $\beta$ -benzoylanilidovinyl, etc.), with a compound selected from those represented by the following general formula:



wherein R<sub>1</sub> and Q have the values given above. A particularly useful group of compounds embraced by Formula III are those represented by the following general formula:



70 wherein R<sub>1</sub> has the values given above, R<sub>3</sub> represents a hydrogen atom or a carbalkoxyl group, such as carbo-

3

methoxyl, carbethoxyl, etc. (e.g., a carbalkoxyl group containing from 2 to 3 carbon atoms), and  $R_4$  and  $R_5$  each represents a hydrogen atom or a lower alkyl group, such as methyl, ethyl, etc. The dyes produced by condensing a cyclammonium quaternary salt selected from those of Formula II with a compound of Formula IIIa can be represented by the following general formula:



wherein  $R$ ,  $R_1$ ,  $R_3$ ,  $R_4$ ,  $R_5$ ,  $n$ ,  $d$  and  $Z$  have the values given above.

The condensations of the intermediates of Formula II with the compounds of Formula III (or IIIa) can be accelerated by basic condensing agents, such as the trialkylamines (e.g., triethylamine, tri-*n*-propylamine, triisopropylamine, tri-*n*-butylamine, etc.), N,N-dialkylanilines (e.g., N,N-dimethylaniline, N,N-diethylaniline, etc.), N-alkylpiperidines (e.g. N-methylpiperidine, N-ethylpiperidine, etc.), etc. The condensations can be carried out in the presence of an inert diluent, such as the lower alcohols (e.g., ethanol, *n*-propanol, isopropanol, *n*-butanol, etc.), pyridine, quinoline, 1,4-dioxane, etc. Heat accelerates the condensations although temperatures varying from ambient temperature (ca. 25° C.) to the reflux temperature of the reaction mixture can be employed.

The following examples will serve to illustrate more fully the preparation of the dyes of our invention.

*Example 1.*—2-[*(3*-dicyanomethylene-5,5-dimethyl-1-cyclohexene-1-yl)methylene]-3-methylthiiazolidine



3-methyl-2-thiothiazolidinone (4 g., 1 mol.+200%) and methyl p-toluenesulfonate (7.44 g., 1 mol.+300%) were mixed and gently heated over a free flame and then allowed to cool slowly to room temperature. 3-dicyanomethylene-1,5,5-trimethyl-1-cyclohexene (1.86 g., 1 mol.), triethylamine (5.6 ml., 1 mol.+300%) and pyridine (15 ml.) were then added and the reaction mixture was heated under reflux for ten minutes. The crude dye was precipitated by the addition with stirring of water (100 ml.). The aqueous solution was decanted and the residue boiled with methyl alcohol (50 ml.) and then chilled overnight. The crude product was filtered off and twice recrystallized from ethyl alcohol. The yield of purified dye was 1.28 g. (46%), M.P. 161-2° C.

*Example 2.*—2-[*(3-dicyanomethylene-5,5-dimethyl-1-cyclohexen-1-yl)-methylene*]-3-methylbenzoxazoline.



2-methylmercaptobenzoxazole (4.95 g., 1 mol. + 200%) and methyl p-toluenesulfonate (5.6 g., 1 mol. + 200%) were mixed and heated to reflux over a free flame and then allowed to cool slowly to room temperature. 3-dicyanomethylene-1,5,5-trimethyl-1-cyclohexene (1.86 g., 1 mol.), triethylamine (4.2 ml., 1 mol. + 200%) and pyri-

4

dine (15 ml.) were added and the reaction mixture heated under reflux for ten minutes. The crude dye was precipitated by the addition with stirring of methyl alcohol (100 ml.). After chilling overnight, the crude dye was filtered off, washed with methyl alcohol and dried. After two recrystallizations from pyridine and methyl alcohol, the yield of pure dye was 2.16 g., (68%), M.P. 168-9°C.

**Example 3.**—2-[*(3-dicyanomethylene - 5,5 - dimethyl-1-cyclohexen-1-yl)-methylene]-3-methylbenzothiazoline.*



20 3-dicyanomethylene - 1,5,5 - trimethyl - 1 - cyclohexene  
 (1.86 g., 1 mol.), 3-methyl-2-methylmercaptobenzothiazolium p-toluenesulfonate (7.34 g., 1 mol.+100%) and triethylamine (2.8 ml., 1 mol.+100%) were dissolved in pyridine (15 ml.) and heated under reflux for ten minutes. The crude dye was precipitated by the addition with stirring of methyl alcohol (100 ml.). After chilling overnight, the crude dye was filtered off, washed with methyl alcohol and dried. After two recrystallizations from pyridine and methyl alcohol, the yield of purified dye was 2.30 g. (69%). M.P. 198-9° C.

*Example 4.*—2-[*(3*-dicyanomethylene-5,5-dimethyl-1-cyclohexen-1-yl)-methylene]-3-methylbenzoselenazolines.



3-dicyanomethylene - 1,5,5 - trimethyl - 1 - cyclohexene (0.93 g., 1 mol.), 3-methyl-2-methylmercaptobenzoselenazolium p-toluenesulfonate (2.07 g., 1 mol.) and triethylamine (1.4 ml., 1 mol.+100%) were dissolved in pyridine (10 ml.) and heated under reflux for ten minutes. The crude dye was thrown out of solution by the addition with stirring of methyl alcohol (100 ml.). After chilling overnight, the crude dye was filtered off, washed with methyl alcohol and dried. The yield of purified dye after two recrystallizations from ethyl alcohol was 0.89 g. (47%), M.P. 183-4° C.

**Example 5.**—2-[*(3-dicyanomethylene - 5,5 - dimethyl-1-cyclohexen-1-yl)-methylene*] - 1 - methylnaphtho[1,2]thiazoline.



3-dicyanomethylene - 1,5,5, - trimethyl - 1 - cyclohexene (0.93 g., 1 mol.), 1-methyl-2-methylmercaptonaphtho[1,2]thiazolium p-toluenesulfonate (2.09 g., 1 mol.) and triethylamine (1.4 ml., 1 mol.+100%) were dissolved in pyridine (15 ml.) and the mixture heated under reflux for ten minutes. The crude dye was thrown out of solution by the addition with stirring of methyl alcohol (100 ml.). After chilling overnight, the crude dye was filtered off, washed with methyl alcohol and dried. The yield of purified dye after three recrystallizations from pyri-

5

dine and methyl alcohol, was 1.45 g., (77%), M.P. 243-4° C. with dec.

Example 6.—2-[3-dicyanomethylene - 5,5 - dimethyl-1-cyclohexen-1-yl)-methylene]-1-ethyl-1,2-dihydroquino-line



3-dicyanomethylene - 1,5,5 - trimethyl - 1 - cyclohexene (1.86 g., 1 mol.), 1-ethyl-2-phenylmercaptoquinolinium p-toluenesulfonate (4.37 g., 1 mol.) and triethylamine (1.4 ml., 1 mol.) were dissolved in pyridine (15 ml.) and heated under reflux for ten minutes. The crude dye was thrown out of solution by the addition with stirring of methyl alcohol (100 ml.). After chilling overnight, the crude dye was filtered off, washed with a little methyl alcohol and dried. The yield of purified dye after two recrystallizations from ethyl alcohol was 1.10 g. (31%), M.P. 203-4° C. with dec.

Example 7.—4-[3-dicyanomethylene - 5,5 - dimethyl-1-cyclohexen-1-yl)-methylene]-1-ethyl-1,4-dihydroquino-line



3-dicyanomethylene-1,5,5-trimethyl-1-cyclohexene (0.93 g., 1 mol.), 1-ethyl-4-phenylmercaptoquinolinium p-toluenesulfonate (2.19 g., 1 mol.) and triethylamine (1.4 ml., 1 mol.+100%) were dissolved in pyridine (10 ml.) and heated under reflux for ten minutes. The crude product was thrown out of solution by the addition with stirring of methyl alcohol (100 ml.). After chilling overnight, the crude dye was filtered off, washed with a little methyl alcohol and dried. After two recrystallizations from methyl alcohol, the yield of purified dye was 0.70 g. (41%), M.P. 163-4° C.

Example 8.—2-[3-dicyanomethylene-5,5-dimethyl-1-cyclohexen-1-yl)-methylene]-1,3-diethylbenzimidazoline



3 - dicyanomethylene - 1,5,5 - trimethyl - 1 - cyclohexene (1.86 g., 1 mol.), 1,3-diethyl-2-ethylmercapto-benzimidazolium p-toluenesulfonate (4.06 g., 1 mol.) and triethylamine (2.8 ml., 1 mol.+100%) were dissolved in pyridine (20 ml.) and heated under reflux for ten minutes. The crude dye was thrown out of solution by the addition with stirring of water (100 ml.). The aqueous solution was then decanted and the residue stirred with methyl alcohol until it became crystalline. After chilling overnight, the crude dye was filtered off, washed with a little methyl alcohol and dried. After two recrystallizations from ethyl alcohol, the yield of purified dye was 0.39 g. (11%), M.P. 195-6° C. with dec.

6

Example 9.—2-[3-dicyanomethylene-5,5-dimethyl-1-cyclohexen-1-yl)-methylene]-1-phenylpyrrolidine



3 - dicyanomethylene - 1,5,5 - trimethyl - 1 - cyclohexene (1.86 g., 1 mol.), 2-methylmercapto-1-phenylpyrrolidinium p-toluenesulfonate (3.63 g., 1 mol.) and triethylamine (2.8 ml., 1 mol.+100%) were dissolved in pyridine (15 ml.) and heated under reflux for fifteen minutes. The crude product was thrown out of solution by the addition with stirring of water (100 ml.). The aqueous solution was decanted and the residue stirred with methyl alcohol until crystalline, chilled overnight and the crude product filtered off and dried. After two recrystallizations from ethyl alcohol, the yield of purified dye was 0.78 g., (23%), M.P. 224-6° C.

Example 10.—2-[3-dicyanomethylene-5,5-dimethyl-1-cyclohexen-1-yl)allylidene]-3-ethylbenzoxazoline



3 - dicyanomethylene - 1,5,5 - trimethyl - 1 - cyclohexene (1.86 g., 1 mol.), 2-β-acetanilidovinyl-3-ethylbenzoxazolium iodide (4.34 g., 1 mol.) and triethylamine (2.8 ml., 1 mol.+100%) were dissolved in pyridine (15 ml.) and heated under reflux for ten minutes. The product was thrown out of solution by the addition with stirring of methyl alcohol (100 ml.). After chilling overnight, the crude dye was filtered off, washed with methyl alcohol and dried. After two recrystallizations from pyridine and methyl alcohol, the yield of pure dye was 2.20 g., (64%), M.P. 224-5° C. with dec.

Example 11.—2-[3-dicyanomethylene-5,5-dimethyl-1-cyclohexen-1-yl)allylidene]-3-ethylbenzothiazoline



3 - dicyanomethylene - 1,5,5 - trimethyl - 1 - cyclohexene (1.15 g., 1 mol.), 2-β-acetanilidovinyl-3-ethylbenzothiazolium iodide (4.50 g., 1 mol.) and triethylamine (2.8 ml., 1 mol.+100%) were dissolved in pyridine (15 ml.) and heated under reflux for ten minutes. The crude dye was thrown out of solution by the addition with stirring of methyl alcohol, the mixture chilled overnight and the crude dye filtered off, washed with methyl alcohol and dried. After two recrystallizations from pyridine and methyl alcohol, the yield of pure dye was 2.61 g. (71%), M.P. 230-1° C. with dec.

Example 12.—2-[3-dicyanomethylene-5-methyl-1-cyclohexen-1-yl]-methylene]-3-methylbenzoxazoline



3-dicyanomethylene-1,5-dimethyl-1-cyclohexene (0.86 g., 1 mol.), 3-methyl-2-methylmercaptobenzoxazolium p-toluenesulfonate (6.72 g., 1 mol.+100%) and triethylamine (2.8 ml., 1 mol.+300%) were dissolved in pyridine (15 ml.) and heated under reflux for ten minutes. The crude dye was thrown out of solution by the addition with stirring of water (50 ml.). The aqueous solution was decanted and the residue stirred with methyl alcohol until crystalline. After chilling overnight, the crude dye was filtered off, washed with methyl alcohol and dried. After two recrystallizations from pyridine and methyl alcohol, the yield of pure dye was 0.94 g. (62%), M.P. 252-3° C. with dec.

Example 13.—2-[3-dicyanomethylene-1-cyclohexen-1-yl]-methylene]-3-methylbenzothiazoline



3-dicyanomethylene-1-methyl-1-cyclohexene (0.79 g., 1 mol.), 3-methyl-2-methylmercaptobenzothiazolium p-toluenesulfonate (3.67 g., 1 mol.+100%) and triethylamine (1.4 ml., 1 mol.+100%) were dissolved in pyridine (10 ml.) and heated under reflux for ten minutes. The crude dye was thrown out of solution by the addition with stirring of water (100 ml.). The aqueous solution was decanted and the residue stirred with methyl alcohol until crystalline. After chilling overnight, the crude dye was filtered off, washed with methyl alcohol and dried. After two recrystallizations from pyridine and methyl alcohol, the yield of pure dye was 0.79 g. (52%), M.P. 256-7° C. with dec.

Example 14.—2-[3-dicyanomethylene-1-cyclohexen-1-yl]-methylene]-3-methylbenzoxazoline



This dye was made in 47% yield by the method of the previous example by using 3-methyl-2-methylmercaptobenzoxazolium p-toluenesulfonate in place of the benzothiazolium salt, M.P. 283-5° C. with dec.

Example 15.—2-[3-(3-dicyanomethylene-1-cyclohexen-1-yl)allylidene]-3-ethylbenzothiazoline



3-dicyanomethylene-1-methyl-1-cyclohexene (0.79 g., 1 mol.), 2-β-acetanilidovinyl-3-ethylbenzothiazolium iodide (2.25 g., 1 mol.) and triethylamine (1.4 ml., 1 mol.+100%) were dissolved in pyridine (10 ml.) and heated under reflux for ten minutes. The crude dye was thrown out of solution by the addition with stirring of water (100 ml.). The aqueous solution was decanted and the residue dissolved in a little methyl alcohol and chilled with occasional stirring for one week. The crude dye was then filtered off, washed with a little methyl alcohol and dried. After two recrystallizations from pyridine and methyl alcohol, the yield of pure dye was 0.65 g. (31%), M.P. 185-6° C. with dec.

dide (2.25 g., 1 mol.) and triethylamine (1.4 ml., 1 mol.+100%) were dissolved in pyridine (15 ml.) and heated under reflux for ten minutes. The reaction mixture was precipitated with water and the aqueous portion decanted.

5 The residue was stirred with methyl alcohol (20 ml.) until crystalline, chilled, filtered and the crude dye washed with methyl alcohol and dried. After two recrystallizations from pyridine and methyl alcohol, the yield of purified dye was 0.72 g. (42%), M.P. 253-4° C. with dec.

10 Example 16.—2-[6-carbethoxy-3-dicyanomethylene-1-cyclohexen-1-yl)methylene]-3-methylbenzoxazoline



6-carbethoxy-3-dicyanomethylene-1-methyl-1-cyclohexene (1.15 g., 1 mol.), 3-methyl-2-methylmercaptobenzoxazolium p-toluenesulfonate (7.02 g., 1 mol.+300%) and triethylamine (2.8 ml., 1 mol.+300%)

15 were dissolved in pyridine (10 ml.) and heated under reflux for ten minutes. The crude dye was then precipitated by the addition of water (100 ml.) and the aqueous solution carefully decanted. The dye failed to crystallize on stirring with methyl alcohol, and was again precipitated with water and then stirred twice with low boiling ligroin. The dye was dissolved in methyl alcohol and chilled for a week with occasional stirring. The crystalline dye was then filtered off and dried. After two crystallizations from methanol, the yield of purified dye was

20 0.24 g. (13%), M.P. 177-8° C. with dec.

Example 17.—2-[6-carbethoxy-3-dicyanomethylene-1-cyclohexen-1-yl)methylene]-3-methylbenzothiazoline



This dye (M.P. 214-15° C. with dec.) was prepared in 68% yield by the method of the preceding example by substituting 3-methyl-2-methylmercaptobenzothiazolium p-toluenesulfonate for the benzoxazolium salt.

Example 18.—2-[3-(6-carbethoxy-3-dicyanomethylene-1-cyclohexen-1-yl)allylidene]-3-ethylbenzothiazoline



6-carbethoxy-3-dicyanomethylene-1-methyl-1-cyclohexene (1.15 g., 1 mol.), 2-β-acetanilidovinyl-3-ethylbenzothiazolium iodide (2.25 g., 1 mol.) and triethylamine (1.4 ml., 1 mol.+100%) were dissolved in pyridine (10 ml.) and heated under reflux for ten minutes. The crude dye was thrown out of solution by the addition with stirring of water (100 ml.). The aqueous solution was decanted and the residue dissolved in a little methyl alcohol and chilled with occasional stirring for one week. The crude dye was then filtered off, washed with a little methyl alcohol and dried. After two recrystallizations from pyridine and methyl alcohol, the yield of pure dye was 0.65 g. (31%), M.P. 185-6° C. with dec.

9

Example 19.—2-[3-(1-carbethoxy-1-cyanomethylene)-5,5-dimethyl-1-cyclohexen-1-yl]methylenec-3-methylbenzothiazoline



3-(1-carbethoxy-1-cyanomethylene)-1,5,5-trimethyl-1-cyclohexene (2.33 g., 1 mol.), 3-methyl-2-methylmercaptobenzothiazolium p-toluenesulfonate (4.04 g., 1 mol. +10%) and triethylamine (2.8 ml., 1 mol. +100%) were dissolved in pyridine (15 ml.) and heated under reflux for ten minutes. The crude dye was precipitated by the addition with stirring of water (100 ml.). The aqueous solution was decanted and the residue stirred with methyl alcohol until crystalline. After chilling overnight, the crude dye was filtered off, washed with a little methyl alcohol and dried. After two recrystallizations from ethyl alcohol, the yield of pure dye was 1.12 g. (30%), M.P. 179-180° C. with dec.

Example 20.—8-[3-dicyanomethylene-5,5-dimethyl-1-cyclohexen-1-yl]methylenec-9-methylacenaphtho[1,2]thiazoline



9-methyl-8-methylmercaptocacenaphtho[1,2]thiazolium p-toluenesulfonate (2.2 g., 1 mol.), 3-dicyanomethylene-1,5,5-trimethyl-1-cyclohexene (0.93 g., 1 mol.) and triethylamine (1.4 ml., 2 mol. +100%) were dissolved in pyridine (20 ml.) and heated under reflux for ten minutes. After chilling, the crude dye was filtered off, washed with water and methyl alcohol and dried. After two recrystallizations from pyridine and methyl alcohol, the yield of pure dye was 0.7 g. (34%), M.P. 193-4° C. with dec.

The intermediates selected from those represented by Formulas III and IIIa can advantageously be prepared by the method of Widequist ("Acta. Chem. Scand.", vol. 3, pp. 303-304, 1949) by condensing a 3-methyl-2-cyclohexen-1-one with an intermediate of the formula:

IV.



wherein R<sub>1</sub> has the values given above. Useful cyclohexeneones include those represented by the following general formula:

V.



wherein R<sub>3</sub>, R<sub>4</sub> and R<sub>6</sub> each have the values given above. Typical intermediates of Formula IV include malononitrile, methyl cyanoacetate, ethyl cyanoacetate, etc. Typical intermediates of Formula V include isophorone, 3,5-dimethyl-2-cyclohexen-1-one, 3-methyl-2-cyclohexen-1-one, 4-carbethoxy-3-methyl-2-cyclohexen-1-one, etc. The following examples will serve to illustrate the preparation of the intermediates of Formula III and IIIa.

Example 21.—3-dicyanomethylene-1,5,5-trimethyl-1-cyclohexene



5

Malononitrile (19.8 g., 1 mol.) and isophorone (46 g., 1 mol. +10%) were dissolved in chloroform and ammonium acetate (2.5 g.) and acetic acid (4 ml.) were added. The mixture was then heated under reflux for one hour in a system fitted for continuous removal of water. The chloroform solution was then washed with two 100 ml. portions of water and the chloroform removed by distillation. The residue was then distilled under vacuum yielding 30.2 g. (54%), B.P. 175-6° C./19 mm., M.P. 79-80° C.

Example 22.—3-(1-carbethoxy-1-cyanomethylene)1,5,5-trimethyl-1-cyclohexene



25

Ethyl cyanoacetate (34 g., 1 mol.) and isophorone (46 g., 1 mol. +10%) were dissolved in chloroform and ammonium acetate (2.5 g.) and acetic acid (4 ml.) were added. The reaction mixture was then heated under reflux for eighteen hours in a system fitted for the continuous removal of water. The chloroform solution was then washed with two 100 ml. portions of water and then the chloroform was removed by distillation. The residue was then distilled under vacuum. The yield of product was 18 g. (26%), B.P. 175-180° C./15 mm.

Example 23.—3-dicyanomethylene-1,5-dimethyl-1-cyclohexene



45

3,5-dimethyl-2-cyclohexen-1-one (12.4 g., 1 mol.) and malononitrile (7.3 g., 1 mol. +10%) were dissolved in chloroform and ammonium acetate (2.5 g.) and acetic acid (4 ml.) were added. The reaction mixture was then heated under reflux for twenty hours in an apparatus designed for the continuous removal of water. The chloroform solution was then washed with two 20 ml. portions of water and the chloroform removed by distillation. The residue was then distilled under reduced pressure yielding 15.1 g. (87%) of purified product, B.P. 170-175° C./18 mm., M.P. 55-7° C.

Example 24.—3-dicyanomethylene-1-methyl-1-cyclohexene



65

3-methyl-2-cyclohexen-1-one (22 g., 1 mol.) and malononitrile (14.5 g., 1 mol. +10%) were dissolved in chloroform (60 ml.) and ammonium acetate (2.5 g.) and acetic acid (4 ml.) were added. The reaction mixture was heated under reflux for four hours in an apparatus

designed for the continuous removal of water. The chloroform solution was then washed with two 25 ml. of water. After removal of the chloroform by distillation, the residue became crystalline. After recrystallization from methyl alcohol, the yield of purified product was 25.5 g. (81%), M.P. 75-6° C.

*Example 25.—6-carbethoxy-3-dicyanomethylene-1-methyl-1-cyclohexene*



4-carbethoxy-3-methyl-2-cyclohexen-1-one (18.1 g., 1 mol.) and malononitrile (7.3 g., 1 mol. + 10%) were dissolved in chloroform (40 ml.) and ammonium acetate (2.5 g.) and acetic acid (4 ml.) were added. The reaction mixture was then heated under reflux for four hours in an apparatus designed for the continuous removal of water. The chloroform solution was then washed with two 25 ml. portions of water and the chloroform removed by distillation. The residue was then distilled under vacuum yielding 15.6 g. (68%) of product, B.P. 200-201° C./9 mm.

All of the dyes of our invention are particularly useful in manufacturing photographic, silver halide emulsions, serving to alter the sensitivity thereof. Sensitization by means of our new dyes is, of course, directed primarily to the ordinarily employed, gelatino-silver-halide, developing-out emulsions. The dyes are advantageously incorporated in the washed, finished emulsion and should, of course, be uniformly distributed throughout the emulsion. In the preparation of photographic emulsions containing our new dyes, it is only necessary to disperse the dyes in the emulsions. The methods of incorporating dyes in emulsion are simple and well known to those skilled in the art of emulsion making. It is convenient to add the dyes from solutions in appropriate solvents. The solvent must, of course, be compatible with the emulsion and substantially free from any deleterious effect on the light-sensitive materials. Pyridine has proven satisfactory as a solvent for the majority of our new dyes.

The concentration of our new dyes in the emulsion can vary widely, i.e., from about 5 to about 100 mgs. per liter of flowable emulsion. The concentration of the dye will vary according to the type of light-sensitive material in the emulsion and according to the effects desired. The suitable and most economical concentration for any given emulsion will be apparent to those skilled in the art upon making the ordinary tests and observations customarily used in the art of emulsion making.

To prepare a gelatino-silver-halide emulsion sensitized with one of our new dyes, the following procedure is satisfactory: A quantity of the dye is dissolved in pyridine or other suitable solvent and a volume of this solution (which may be diluted with methanol) containing from 5 to 100 mgs. of dye is slowly added to about 1000 cc. of a gelatino-silver-halide emulsion, with stirring. Stirring is continued until the dye is uniformly distributed throughout the emulsion. With most of our new dyes, 10 to 20 mgs. of dye per liter of emulsion suffices to produce the maximum sensitizing effect with the ordinary gelatino-silver-bromide (including bromide) emulsions. With fine-grain emulsions, which include most of the ordinarily employed gelatino-silver-chloride emulsions, somewhat larger concentrations of dye may be necessary to secure the optimum sensitizing effect.

The above statements are only illustrative and are not to be understood as limiting our invention in any sense, as it will be apparent that our new dyes can be incorporated by other methods in many of the photographic silver halide emulsions customarily employed in the art. For

instance, the dyes can be incorporated by bathing a plate or film upon which an emulsion has been coated, in the solution of the dye, in an appropriate solvent. Bathing methods, however, are not to be preferred ordinarily.

Photographic silver halide emulsions which can advantageously be sensitized by means of the new dyes of our invention comprise the customarily employed gelatino-silver-chloride, gelatino-silver-chlorobromide, gelatino-silver-bromide, and gelatino-silver bromide developing-out emulsions.

Photographic silver halide emulsions, such as those listed above, containing the sensitizing dyes of our invention can also contain such addenda as chemical sensitizers, e.g., sulfur sensitizers (e.g., allyl thiocarbamide, thiourea, allylisothiocyanate, cystine, etc.), various gold compounds (e.g., potassium chloroaurate, auric trichloride, etc.) (see U.S. Patents 2,540,085; 2,597,856 and 2,597,915), various palladium compounds, such as palladium chloride (U.S. 2,540,086), potassium chloropalladate (U.S. 2,598,079), etc., or mixtures of such sensitizers; anti-foggants, such as ammonium chloroplatinate (U.S. 2,566,245), ammonium chloroplatinite (U.S. 2,566,263), benzotriazole, nitrobenzimidazole, 5-nitroindazole, benzidine, mercaptans, etc. (see Mees, "The Theory of the Photographic Process," Macmillan Pub., page 460), or mixtures thereof; hardeners, such as formaldehyde (U.S. 1,763,533), chrome alum (U.S. 1,763,533), glyoxal (U.S. 1,870,354), dibromacrolein (Br. 406,750), etc.; color couplers, such as those described in U.S. Patent 2,423,730, Spence and Carroll U.S. Patent 2,640,776, etc.; or mixtures of such addenda. Dispersing agents for color couplers, such as those set forth in U.S. Patents 2,322,027 and 2,304,940, can also be employed in the above-described emulsions.

In the manner described above, a number of the dyes of our invention represented by Formula I above were separated incorporated in an ordinary gelatino-silver-halide emulsion, the dyes being thoroughly incorporated in the emulsions by stirring. After a short digestion, the emulsions were coated onto ordinary cellulose acetate film supports and the coatings exposed in a spectrograph and sensitometer, and then developed in the usual way. The type of emulsion (silver-chlorobromide or silver-bromide), sensitizing range, and maximum absorption for each of the dyes are indicated in the following table.

|    | Dye of Example | Emulsion | Sensitizing Range in mu | Maximum in mu |
|----|----------------|----------|-------------------------|---------------|
| 1  | ClBr           | to 570   | 540                     |               |
| 2  | BrI            | to 610   | 570                     |               |
| 3  | BrI            | to 650   | 600                     |               |
| 4  | BrI            | to 650   | 610                     |               |
| 5  | BrI            | to 650   | 610                     |               |
| 6  | ClBr           | 530-690  | 655                     |               |
| 7  | BrI            | 600-725  | 690                     |               |
| 8  | BrI            | 500-590  | 640                     |               |
| 9  | ClBr           | 440-540  | 480                     |               |
| 10 | BrI            | 590-695  | 670                     |               |
| 11 | BrI            | 560-750  | 685                     |               |
| 12 | BrI            | to 585   | 560                     |               |
| 13 | BrI            | to 630   | 600                     |               |
| 14 | ClBr           | 445-595  | 640                     |               |
| 16 | BrI            | to 620   | 600                     |               |
| 17 | BrI            | to 630   | 580                     |               |
| 18 | BrI            | 560-770  | 720                     |               |
| 19 | BrI            | to 630   | 600                     |               |
| 20 | BrI            | 530-650  | 620                     |               |

The 2-methylmercapto-1-phenylpyrrolidinium p-toluenesulfonate employed in Example 9 above was prepared as follows: 1-phenyl-2-thiopyrrolidone (1.77 g., 1 mol.) and methyl p-toluenesulfonate (1.86 g., 1 mol. + 50%) were fused and heated on a steam bath for one hour. The solid quaternary salt was used in dye condensations without further purification.

The 1-phenyl-2-thiopyrrolidone used above was prepared as follows: 1-phenyl-2-pyrrolidone (26 g., 1 mol.) [Späth and Lintner Ber., 69B, 2727 (1936)] and phosphorous pentasulfide (18 g., 1 mol. + 50%) were dissolved in pyridine (100 ml.) and heated to reflux. After ten minutes the reaction mixture was poured into water

13

(1000 ml.) with stirring. The oily product was extracted with ether and the ethereal solution concentrated and the residue distilled at 195-197° C./8 mm. After recrystallization of the solid distillate from ethanol, the yield of pale yellow crystals was 17 g. (59%), M.P. 73-5° C.

The copending application of J. E. Jones Serial No. 586,054, filed on even date herewith (now U.S. Patent 2,860,982, issued November 18, 1958), illustrates wedge spectrograms obtained from photographic silver halide emulsions containing the new dyes of our invention, alone and in combination with certain pyridine bases.

What we claim as our invention and desire secured by Letters Patent of the United States is:

1. A photographic silver halide emulsion sensitized with a polymethine dye selected from those represented by the following general formula:



wherein R represents an alkyl group containing from 1 to 4 carbon atoms, d represents a positive integer of from 1 to 2, and Q represents the atoms necessary to complete a cyclohexene ring.

2. A photographic silver halide emulsion sensitized with a polymethine dye selected from those represented by the following general formula:



wherein R represents an alkyl group containing from 1 to 4 carbon atoms, d represents a positive integer of from 1 to 2, and Q represents the atoms necessary to complete a cyclohexene ring.

3. A photographic silver halide emulsion sensitized with a polymethine dye selected from those represented by the following general formula:



wherein R represents an alkyl group containing from 1 to 4 carbon atoms, d represents a positive integer of from 1 to 2, and Q represents the atoms necessary to complete a cyclohexene ring.

4. A photographic silver halide emulsion sensitized with a polymethine dye selected from those represented by the following general formula:



wherein R represents an alkyl group containing from 1 to 4 carbon atoms, d represents a positive integer of from 1 to 2, and Q represents the atoms necessary to complete a cyclohexene ring.

14

5. A photographic silver halide emulsion sensitized with a polymethine dye selected from those represented by the following general formula:



wherein R represents an alkyl group containing from 1 to 4 carbon atoms, d represents a positive integer of from 1 to 2, and Q represents the atoms necessary to complete a cyclohexene ring.

15 6. A photographic silver halide emulsion sensitized with a polymethine dye selected from those represented by the following general formula:



25 wherein R represents an alkyl group, R1 represents a member selected from the group consisting of a cyano group and a carbalkoxyl group, Q represents the atoms necessary to form a cyclohexene ring, n and d each represents a positive integer of from 1 to 2, and Z represents the non-metallic atoms necessary to complete a heterocyclic nucleus containing from 5 to 6 atoms in the heterocyclic ring.

30 7. A photographic silver halide emulsion sensitized with a polymethine dye selected from those represented by the following general formula:



45 wherein R represents an alkyl group containing from 1 to 4 carbon atoms, R1 represents a member selected from the group consisting of a cyano group and a carbalkoxyl group containing from 2 to 3 carbon atoms, R3 represents a member selected from the group consisting of a hydrogen atom and a carbalkoxyl group containing from 2 to 3 carbon atoms, R4 and R5 each represents a member selected from the group consisting of a hydrogen atom and

50 an alkyl group containing from 1 to 2 carbon atoms, n and d each represents a positive integer of from 1 to 2, and Z represents the non-metallic atoms necessary to complete a heterocyclic nucleus selected from the group consisting of those of the thiazole series, those of the benzothiazole series, those of the naphthothiazole series, those of the thianaphtheno-7',6',4,5-thiazole series, those of the

55 oxazole series, those of the benzoxazole series, those of the naphthoxazole series, those of the selenazole series, those of the benzoselenazole series, those of the naphtho-selenazole series, those of the thiazoline series, those of the 2-quinoline series, those of the 4-quinoline series,

60 those of the 1-isoquinoline series, those of the 3,3-dialkyl-indolenine series, those of the 2-pyridine series, those of the 4-pyridine series, those of the benzimidazole series, those of the pyrrolidine series, and those of the acenaph-

65 thothiophene series, provided that when Z represents the non-metallic atoms necessary to complete a heterocyclic nucleus of the pyrrolidine series, R can additionally represent a monocyclic aryl group of the benzene series.

70 75 8. A photographic silver halide emulsion sensitized with

15

the polymethine dye represented by the following formula:



9. A photographic silver halide emulsion sensitized with the polymethine dye represented by the following formula:



10. A photographic silver halide emulsion sensitized with the polymethine dye represented by the formula:



11. A photographic silver halide emulsion sensitized with the polymethine dye represented by the following formula:



12. A photographic silver halide emulsion sensitized with the polymethine dye represented by the following formula:



16

13. A photographic silver halide emulsion sensitized with a polymethine dye selected from those represented by the following general formula:



- 10 wherein R represents an alkyl group containing from 1 to 4 carbon atoms, R<sub>1</sub> represents a member selected from the group consisting of a cyano group and an alkoxy carbonyl group containing from 2 to 3 carbon atoms, Q represents the non-metallic atoms necessary to complete a cyclohexene ring, n and d each represents a positive integer of from 1 to 2, and Z represents the non-metallic atoms necessary to complete a heterocyclic nucleus selected from the group consisting of those of the thiazole series, those of the benzothiazole series, those of the naphthothiazole series, those of the thianaphtheno-7',6',4,5-thiazole series, those of the oxazole series, those of the benzoxazole series, those of the naphthoxazole series, those of the selenazole series, those of the benzoselenazole series, those of the thiazoline series, those of the 2-quinoline series, those of the 4-quinoline series, those of the 1-isoquinoline series, those of the 3,3-dialkylindolenine series, those of the 2-pyridine series, those of the 4-pyridine series, those of the benzimidazole series, those of the pyrrolidine series 30 and those of the acenaphtho[1,2,1-thiazole series, provided that when Z represents the non-metallic atoms necessary to complete a heterocyclic nucleus of the pyrrolidine series, R can additionally represent a monocyclic aryl group of the benzene series.

**References Cited in the file of this patent**

UNITED STATES PATENTS

- |           |                 |               |
|-----------|-----------------|---------------|
| 2,282,116 | Brooker         | May 5, 1942   |
| 2,455,420 | Kendall et al.  | Dec. 7, 1948  |
| 2,697,707 | Kendall et al.  | Dec. 21, 1954 |
| 2,721,799 | Edwards et al.  | Oct. 25, 1955 |
| 2,756,227 | Heseltine       | July 24, 1956 |
| 2,766,233 | Kartinos et al. | Oct. 9, 1956  |
| 2,773,869 | Leavitt         | Dec. 11, 1956 |

#### OTHER REFERENCES

- Chemical Abstracts, 16, 3101 (abstract of Brit. Med. Journal, 1922 I, 514-5).  
Chemical Abstracts, 19, 530 (abstract of Proc. Roy. Soc., London, 96B, 317-33, 1924).

UNITED STATES PATENT OFFICE  
Certificate of Correction

April 14, 1959

Patent No. 2,882,158

Leslie G. S. Brooker et al.

It is hereby certified that error appears in the printed specification of the above numbered patent requiring correction and that the said Letters Patent should read as corrected below.

Column 2, line 9, for "(e.g., pyridine" read —(e.g., pyridine—; column 6, line 66, Example 11, second line below the formula, for "(1.15 g., 1 mol.)" read —(1.86 g., 1 mol.)—; column 10, line 34, Example 22, fourth line below the formula, for "other" read —then—; column 11, line 49, for "sensiitve" read —sensitive—; column 12, line 36, for "separated" read —separately—; line 41, for "sensitometer" read —sensitometer—; column 15, lines 3 to 9 inclusive, the left-hand portion of the formula should appear as shown below instead of as in the patent:



column 16, lines 5 to 8 inclusive, the formula should appear as shown below instead of as in the patent:



Signed and sealed this 13th day of October 1959.

[SIMAL]

Attest:

KARL H. AXLINE,  
Attesting Officer.

ROBERT C. WATSON,  
Commissioner of Patents.